# EUROPEAN PATENT SPECIFICATION

(11) **EP 0 123 224 B1**
(45) Date of publication and mention of the grant of the patent: **29.06.1988**
(21) Application number: 84104136.1
(22) Date of filing: 12.04.1984
(51) Int. Cl.: G03C 1/76, G03C 1/52

(54) **Heat sensitive recording materials**
Wärmeempfindliche Aufzeichnungsmaterialien
Matériaux pour l'enregistrement thermosensible

(30) Priority: 13.04.1983 JP 65043/83; 24.06.1983 JP 114752/83; 30.08.1983 JP 158469/83; 13.09.1983 JP 169015/83
(43) Date of publication of application: 31.10.1984
(73) Proprietor: FUJI PHOTO FILM CO., LTD., Kanagawa 250-01 (JP)
(72) Inventor: Usami, Toshimasa, Fujinomiya-shi Shizuoka (JP); Tanaka, Toshiharu, Fujinomiya-shi Shizuoka (JP); Shinozaki, Fumiaki, Fujinomiya-shi Shizuoka (JP)
(74) Representative: Patentanwälte Dr. Solf & Zapf

(56) References cited:
- DE-A- 2 341 113
- DE-A- 3 221 643
- US-A- 3 202 510

## Description

### Field of the Invention

This invention relates to the preparation of heat-sensitive recording materials, and particularly the preparation of fixable diazo heat-sensitive recording materials. More particularly, the invention relates to a process for preparing a heat-sensitive recording material comprising a support having thereon a recording layer containing (a) a diazo compound, (b) a coupling component and (c) a coloring activator, wherein at least one of said diazo compound (a), said coupling component (b) and said coloring activator (c)a is present in microcapsules as the core material with the provisio that all three components (a) to (c) are not present in the same microcapsules, and the wall of said microcapsules being formed of a polymer, said heat-sensitive recording material having excellent shelf life before heat recording, provide high coloring density as a result of heat recording and can be fixed by light after heat recording.

### Background of the Invention

A heat sensitive recording method has the advantages that (1) development is unnecessary, (2) when the support of the heat sensitive material is paper, the characteristics of the paper are similar to those of paper in general, (3) handling is easy, (4) a coloring density is high, (5) the recording device is simple and inexpensive, (6) noise is not generated on recording, and hence the heat sensitive recording method is being widely used in facsimile and printer fields.

Heat sensitive. recording materials for the recording method include predominantly a leuco coloring type heat sensitive recording material with excellent coloring density and coloring speed. However, a leuco coloring type heat sensitive recording material has the disadvantages that the recording material is colored on handling, heating, or solvent treatment although after recording to stain the recorded images and also the recorded color images disppear due to the action of plasticizers present in adhesive tape.

For preventing formation of color in a leuco coloring type heat sensitive recording material by careless handling, addition of a granular wax (JP-B-14,531/1975) has been proposed and also for preventing permeation of plasticizers, formation of a protective layer on the recording layer of the recording material (JP-A-125,354/1981) was proposed.

However, the foregoing techniques are still unsatisfactory. In particular, these techniques cannot be used for the purpose of preventing the falsification or alterations after recording. Hence an improvement in these techniques has been keenly desired.

A method of using a heat sensitive recording material composed of a diazo compound, a coupling component, and an alkali generating agent or a coloring assistant and irradiating the recording material with light after heat recording to decompose the unreacted diazo compound, whereby further coloring of the recording material is stopped is known as a method of stopping coloring of unnecessary areas of a heat sensitive recording material after heat recording.

However, in a heat sensitive recording material, sometimes during the storage of the recording material, a coupling reaction gradually proceeds to form undesirable coloring (fog). Therefore, prevention of contact of the coloring components with each other to eliminate the occurrence of the coupling reaction by containing at least one of the coloring components in the form of discontinuous particles (solid dispersion) is attempted. However, this attempt has the disadvantages that the shelf life of the recording material is still insufficient and also coloring on heating is reduced.

As an alternative approach, it is known to place the diazo compound and the coupler component in different layers to minimize the contact of the components. This technique may improve the shelf life of the recording material but since the heat coloring property is reduced and the recording material cannot respond to high-speed recording with short pulse width, the technique is unsuitable for practical use.

Furthermore, a method of satisfying both the shelf life and the heat coloring property of heat sensitive recording materials involving isolating (soluting) one of the coupling component and the coloring assistant from the other components by encapsulating the component with a nonpolar waxy material (JP-A-4414/ 1982 and 142,636/1982) or hydrophobic polymer (JP-A-192,944/1982) is known. In the foregoing encapsulationg methods, a waxy material of hydrophobic polymer is dissolved in a solvent, a coloring compnent is dissolved or dispersed in the solution, and then the solvent is evaporated off to form microcapsules containing the coloring component. However, in using the encapsulation method, the coloring component is incompletely encapsulated as the core material of the microcapsules and is uniformly mixed with the encapsulating material of the microcapsules. Thus, pre-coupling gradually proceeds at the interface of the walls of the microcapsules during storage of the recording material and hence the shelf life of the recording material is not satisfactory. Also, in the technique, the walls of the microcapsules must be fused by heating for performing the coloring reaction, which results in a reduction in the heat coloring property. Furthermore, in the foregoing method, there is the difficult problem that after forming the microcapsules, the solvent used for dissolving the waxy material of the hydrophobic polymer must be removed and hence the foregoing method is still unsatisfactory in this point.

From DE-A-23 41 113 and 32 21 643 there are known heat-sensitive recording materials comprising a support having thereon a recording layer containing a diazo compound, a coupling component and a coloring activator wherein at least one of these components is present in microcapsules as the color material with the provisio that not all of these three components are present in the same microcapsules and the wall of that microcapsules being formed of a polymer. However, in these known processes the capsule walls are made from preformed polymers rather than by polymerisation of a polymer-forming reactant or reactants at the time of encapsulation. However, in practice it has been shown that the shelf life of the capsules prepared according the known processes is not sufficient.

The object of the present invention therefore is to prepare a heat-sensitive recording material having an improved shelf life and being capable of stopping the formation of coloring in unnecessary areas.

As the result of various investigations it has now been found that the above object of this invention is attained by forming the wall of the microcapsules by a polymerization reaction around the core material.

Subject-matter of the present invention is a process for preparing a heat sensitive recording material comprising a support having thereon a recording layer containing (a) a diazo compound, (b) a coupling component and (c) a coloring activator, wherein at least one of said diazo compound (a), said coupling component (b) and said coloring activator (c) is present in microcapsules as the core material with the provisio that all three components (a) to (c) are not present in the same microcapsules, and the wall of said microcapsules is formed of a polymer, which is characterized in that the core material is dispersed in one or more reactants and the obtained dispersion is then subjected to a polymerisation reaction whereby the wall of said microcapsules is formed around the core material.

The heat-sensitive recording material prepared according to the claimed process has an excellent shelf life and high coloring speed and coloring density. It is capable of stopping the formation of coloring in unnecessary areas (hereinafter referred to as "fixing") by photodecomposing unreacted diazo compound after heat recording. In addition, it has an excellent production aptitude.

According to a preferred embodiment of this invention, in the preparation of the heat sensitive recording material, as material of the wall of the microcapsules a polyurethane, polyurea, polyamide or polyester is used.

According to another preferred embodiment of this invention, in the obtained heat sensitive recording material, the core materials are present in the microcapsules together with an organic solvent.

According to still another preferred embodiment of this invention, in the obtained heat sensitive recording material, the core material is the diazo compound and the wall of said microcapsules is composed of a polymer formed around the core material by the reaction of polyhydric isocyanate and a polyol.

According to an even further preferred embodiment of this invention, in the obtained heat sensitive recording material, the diazo compound is one represented by the general formula wherein Ar represents a substituted or unsubstituted aromatic moiety and X represents an acid anion containing a perfluoroalkyl group or an acid anion containing a perfluoroalkenyl group.

### Detailed Description of the Invention

The microcapsules prepared according to this invention are not of the type that a coloring reaction occurs upon rupturing of microcapsules by heat or pressure to contact a reactive material present in the microcapsules as the core material and a reactive material present outside the microcapsules as used for conventional recording material but of the type that the core material present in the microcapsules and a reactive material present outside the microcapsules react through the walls of the microcapsules upon heating.

It is known that when the wall of a microcapsule is formed by polymerization, the wall thus formed is not a completely impermeable film but is permeable to some extent. The permeability of the wall of the microcapsule in the above-decribed conventional case results in a low molecular material gradually permeating therethrough over a long period of time. However, the phenomenon that a reactive material permeates instantly through the wall of the microcapsule on heating as in the present invention is not yet known. Accordingly, in the case of the microcapsules in this invention it is necessary to fuse the wall of the microcapsules by heating and the wall may be formed using a polymer having a high melting point, which provides the heat sensitive recording material with excellent shelf life.

In fact, when the core material is removed from the microcapsules prepared according to this invention and the residue is heated the wall of the microcapsules is scarcely fused.

The heat sensitive recording material prepared according to this invention contains (a) a diazo compound, (b) a coupling component and (c) a coloring activator in the recording layer in a form that one or two of these three components are present in microcapsules (when two components are encapsulated, the components may be present in the same microcapsules or in different microcapsules), the wall of the microcapsules being composed of a high molecular weight compound formed in situ around the core material by polymerization after emulsifying the core material in a reactant for the high molecular material.

The diazo compound used in this invention is a diazonium salt represented by general formula (1) wherein Ar represents a substituted or unsubstituted aromatic moiety) N2 represents a diazonium group and X- represents an acid anion, preferably an acid anion containing a perfluoroalkyl group or an acid anion containing perfluroalkenyl group, which can be colored by undergoing a coupling reaction with the coupling component and can be decomposed by light.

The substituted aromatic moiety represented by Ar are, preferably, represented by general formula wherein Y represents a substituted amino group, an alkoxy group having 1 to 18 carbon atoms, an alkylthio group having 1 to 18 carbon atoms, an arylamino group having 6 to 18 carbon atoms, or an acylamino group having 1 to 18 carbon atoms; said. substituted amino group preferably including a dialkylamino group having 1 to 36 carbon atoms, an arylamino group having 6 to 18 carbon atoms, a morpholino group, a piperidino group, a pyrrolidino group, and R represents hydrogen, an alkyl group having 1 to 5 carbon atoms, a halogen atom (e.g., I, Br, Cl, F) an alkoxy group having 1 to 18 carbon atoms, or an arylamino group having 1 to 18 carbon atoms.

Special examples of the diazonium compounds formng salts are 4-diazo-1-dimethylaminobenzene, 4-diazo-1-diethyiaminobenzene, 4-diazo-1-dipropylaminobenzene, 4-diazo-1-dibenzylaminobenzene, 4-diazo-1-dibenzylaminobenzene, 4-diazo-1-ethylhydroxyethylaminobenzene, 4-diazo-1-diethylamino-3-methoxybenzene, 4-diazo-1-dimethylamino-2-methylbenzene, 4-diazo-I-benzylamino-2,5-diethoxybenzene, 4-diazo-1-morpholinobenzene, 4-diazo-1-morpholino-2,5-diethoxybenzene, 4-diazo-1-morpholino-2,5-dibutoxybenzene, 4-diazo-1-anilinobenzene, 4-diazo-1-tolylmercapto-2,5-diethoxybenzene, ₄-diazo-₁,₄-methoxybenzoylamino-2,5-diethoxybenzene.

Special examples of suitable acid anions are CₙF₂ₙ₊₁COO⁻ (wherein N is 3 to 9), CₘF₂ₘ₊₁SO3⁻ (wherein m is 2 to 8), ClF_{2lf1}SO₂)₂CH⁻ (wherein I is 1 to 18),

Of the foregoing acid anions, acid anions having a perfluoroalkyl group or a perfluoroalkenyl group each having less than 20 carbon atoms are preferred since the increase of fog at shelf life of the heat sensitive recording material is less.

Special examples of diazo compounds (diazonium salts) which can be used in this invention are as follows:

The coupling component used in this invention is a compound which forms a dye upon coupling with the diazo compound (diazonium salt) under basic conditions. Specific examples of suitable coupling components are rescorcin, fluoroglucin, sodium 2,3-dihydroxynaphthalene-6-sulfonate, 1-hydroxy-2-naphthoic acid morpholinopropylamide, 1,5-dihydroxynaphthalene, 2,3-dihydroxynaphthalene, 2,3-dihydroxy-6-sulfanilnaphthalene, 2-hydroxy-3-naphthoic acid morpholinopropylamide, 2-hydroxy-3-naphthoic acid anilide, 2-hydroxy-3-naphthoic acid-2'-methylanilide, 2-hydroxy-3-naphthoic acid ethanolamide, 2-hydroxy-3-naphthoic acid octylamide, 2-hydroxy-3-naphthoic acid-N-dodecyl-oxypropyl- amide, 2-hhydroxy-3-naphthoic acid tetradecylamide, acetanilide, acetoacetanilide, benzylacetanilide, 1-phenyl-3-methyl-5-pyrazolone, 1-(2',4',6'-trichlorophenyl)-3-benzamido-5-pyrazolone, 1-(2',4',6'-trichlorophenyl)-3-anilino-5-pyrazolone, 1-phenyl-3-phenylacetamido-5-pyrazolone.

Furthermore, by using two or more of these coupling components, images having a desired hue can be obtained.

A sparingly water-soluble or water insoluble basic material or a material generating an alkali upon heating is used as the coloring activator.

Examples of coloring activators which can be used in this invention include nitrogen-containing compounds such as inorganic and organic ammonium salts, organic amines, amides, urea and derivatives thereof, thiourea and derivatives thereof, thiazoles, pyrroles, pyrimidines, piprazines, guanidines, indoles, imidazoles, imidazolines, triazoles, morpholines, piperidines, amidines, formazines, pyridines.

Specific examples of colouring activators are ammonium acetate, tricyclohexylamine, tribenzylamine, octadecylbenzylamine, stearylamine, allylurea, thiourea, methylthiourea, allylthiourea, ethylenethiourea, 2-benzylimidazole, 4-phenyl-imidazole, 2-phenyl-4-methylimidazole, 2-undecyl-imidazoline, 2,4,5-trifuryl-2-imidazolie, 1,2-diphenyl-4,4-dimethyl-2-imidazoline, 2-phenyl-2-imidazoline, 1,2,3-triphenylguanidine, 1,2- ditolylguanidine, 1,2-dichlorohexylguanidine, 1,2,3-tricyclohexylguanidine, guanidine trichloroacetate, N,N'-dibenzylpiperazine, 4,4'-dithiomorpholine, morpholium trichloroacetate, 2-amino-benzothiazole, 2-benzoylhydrazino-benzothiazole. These coloring activators may be used individually or as a combination thereof.

In this invention, by appropriately selecting the material for and the thickness of the wall of the microcapsules, the core material in the microcapsules may be a solution, or semi-solid, or a solid but a solution is preferred since in this case, the core material immediately permeates or reacts to form color at heat recording. Accordingly, it is preferred to use a high-boiling solvent which is a liquid at normal temperature as the core material in this invention.

In this invention, it is effective for improving the shelf life of the heat sensitive recording material and increasing the coloring speed and coloring density of the recording material to dissolve or disperse the core material in a water-insoluble organic solvent, emulsify the solution or dispersion, and form a microcapsule wall around the core material by polymerization. Organic solvents having a boiling point of higher than about 180°C, such as phosphoric acid esters, phthalic acid esters, other carboxylic acid esters, fatty acid amids, akylated biphenyls, alkylated terphenyls, chlorinated paraffins, alkylated naphthalenes, diarylethanes, are preferred as suitable organic solvents.

Special examples of suitable organic solvents which can be used in this invention are tricresyl phosphate, trioctyl phosphate, octyldiphenyl phosphate, tricyclohexyl phosphate, dibutyl phthalate, dioctyl phthalate, dilauryl phthalate, dicyclohexyl phthalate, butyl oleate, diethylene glycol dibenzoate, dioctyl sebacate, dibutyl sebacate, diocyl adipate, trioctyl trimellitate, acetyltriethyl citrate, octyl maleate, dibutyl maleate, isopropylbiphenyl, isoamylbiphenyl, chlorinated paraffin, diisopropylnaphthalene, 1,1'- ditolylethane, 2,4-di-t-aminophenol, N,N-dibutyl-2-butoxy-5-t-octylaniline. Of these solvents, ester solvents such as dibutyl phthalate, diethyl phthalate, dibutyl maleate, are preferred.

The microcapsules used in this invention are prepared by emulsifying a core material containing a reactive material and then forming a wall of a high molecular weight compound around the oil drops of the core material. In this invention, one or two of the foregoing diazo compound, the coupling component and the coloring activator are present in the microcapsules. When the two components are present in the microcapsules, both components may be present in same microcapsules or may be present in different microcapsules. Furthermore, in this invention, the foregoing three components may be present in different microcapsules or two components are present in the same microcapsules and another component may be present in other microcapsule. However, where the three components are present in the same microcapsules are exlcuded in this invention. Thus, the term "encapsulating at least one of the three components" of this invention means the embodiments described above.

In forming a high-molecular weight material around the droplets of the core material thus formed by emulsification as the wall of the microcapsules, the reactant or reactants forming the high molecular weight material are added to the interior and/or the interior of the oil droplets.

Special examples of high molecular weight compounds thus formed are polyurethane, polyurea, polyamide, polyester, polycarbonate, a urea-formaldehyde resin, a melamine resin, polystyrene, a styrene- methacrylate copolymer, a styrene-acrylate copolymer, gelatin, polyvinyl pyrrollidone, polyvinyl alcohol.

Two or more of the foregoing high molecular weight materials may be employed as the wall materials in this invention. Preferred high molecular weight materials are polyurethane, polyurea, polyamide, polyester, polycarbonate, and polyurethane and polyurea are more preferred.

The high molecular weight material used in this invention has preferably a melting point higher than about 150°C so that the wall is not melted at the temperature of heat recording.

As described above, in this invention, at least one of the diazo compound, the coupling component and the coloring activator which are the main components used in this invention is employed as the core material of the microcapsules. That is, the diazo compound, the coupling component or the coloring activator may be used as the core material; or the diazo compound and the coupling component, the diazo compound and the coloring activator, or the coloring component and the coloring activator may be used as the core material, and in the latter case, another component may be incorporated in the recording layer without being encapsulated. When two components are used as the core material, both components may be present in the same microcapsules or different microcapsules. In this invention, each of the three components may be present in different microcapsule or two components may be present in the same microcapsules and another component is present in other microcapsules.

For forming the wall of the microcapsules in this invention, a microcapsulation method involving polymerization of a reactant from the inside of the droplets of the core material can be effectively used. That is, in this case, microcapsules having a uniform particle size can be obtained in a short period of time and such microcapsules are preferred for a heat sensitive recording material having excellent shelf life.

Specific examples of compounds which can be used in the foregong microcapsulation method are described in, for example, U.S.-A-3,726,804 and 3,796,669.

For example, in using polyurethane as the wall of the microcapsules, a polyvalent isocyanate and a material (e.g., a polyol) forming the microcapsule wall by a reaction with the isocyanate are mixed with an oily solution of the core material, the mixture is dispersed by emulsification in water, and the temperature is increased to cause a polymer-forming reaction at the interface of the oil droplets in the emulsion, whereby the wall of the microcapsules is formed. In this case, a low-boiling auxiliary solvent having a high dissolving power can be used in the oily solution.

The polyisocyanates and polyols used in the above case are described in, for example, U.S.-A-3,135,716; 3,281,383; 3,468,922; 3,773,695; 3,793,268; JP-B-40,347/'73; 24,159/'74; and JP-A-80,191/'73 and 84,086/'73.

Also, in this case, f.i. a tin salt, may be used for promoting the urethane forming reaction.

In forming the microcapsules used in this invention, it is effective for obtaining a heat sensitive recording material having a good shelf life and high coloring speed and high heat coloring property to use a polyhydric isocyanate as a first wall-forming material and a polyol as a second wall-forming material as described above.

Examples of polyhydric isocyanates used as the first wall-forming material are diisocyanates such as m-phenylene diisocyanate, p-phenylene diisocyanate, 2,6-trichiene diisocyanate, 2,4-tolylene diisocyanate, naphthalene-1,4-diisocyanate, diphenylmethane-4,4'-diisocyanate, 3,3'-dimethoxy-4,4'-biphenyl- diisocyanate, 3,3'-dimethyldiphenylmethane-4,4'-diisocyanate, xylylene-1,4-diisocyanate, 4,4'-diphenylpropane diisocyanate, trimethylene diisocyanate, hexamethylene diisocyanate, propylene-1,2-diisocyanate, butylene-1,2-diisocyanate, cyclohexylene-1,2-diisocyanate, cyclohexylene-1,4⁼diisocyanate; triisocyanates such as 4,4',4"-triphenylmethane triisocycyanate, toluene-2,4,6-triisocyanate; tetraisocyanates such as 4,4'-dimethyldiphehylmethane-2,2',5,5'-tetraisocyanate; prepolymers such as an addition product of hexamethylene diisocyanate and trimethylolpropane, an addition product of 2,4-tolylene diisocyanate and trimethylolpropane, an addition product of xylylene diisocyanate and trimethylolpropane, and an addition product of tolylene diisocyanate and hexanetriol.

The polyol used as the second wall-forming material includes aliphatic and aromatic polyhydric alcohols, hydroxy polyesters, hydroxy polyalkylene ethers.

Preferred polyols are polyols having a molecular weight lower than 5,000 and having the following group (I), (II), (III) or (IV) between the two hydroxy groups in the molecular structure;
(I) aliphatic hydrocarbon group having 2 to 8 carbon atoms, In groups (II), (III) and (IV), Ar' represents an unsubstituted or substituted aromatic moiety and the aliphatic hydrocarbon group of (I) has the moiety -CnH2n- wherein n is 2 to 8 as the fundamental skeleton and the hydrogen atom may be replaced by another element.

Specific examples of polyols of group (I) are ethylene glycol, 1,3-propanediol, 1,4-butanediol, 1,5-pentanediol, 1,6-hexanediol, 1,7-heptanediol, 1,8-octanediol, propylene glycol, 2,3-dihydroxybutane, 1,2-dihydroxybutane, 1,3-dihydroxybutane, 2,2-dimethyl-1,3-propanediol, 2,4-pentanediol, 2,5-hexanediol, 3-methyl-1,5-pentanediol, 1,4-cyclohexanedimethanol, dihydroxycyclohexane, dithylene glycol, 1,2,6-trihydroxyhexane, phenylethylene glycol, 1,1,1-trimethyioipropane, hexanetriol, pentaerythritol, glycerol.

Specific examples of polyols of group (II) are the condensation products of aromatic polyhydric alcohols such as 1,4-di-(2-hydroxyethoxy)benzene, resorcinol dihydroxyethyl ether, and alkylene oxides.

Specific examples of polyols of group (III) are p-xylylene glycol, m-xylylene glycol, a,a'-dihydroxy-p-diisopropylbenzene.

Specific examples of polyols of group (IV) are 4,4'-dihydroxydiphenylmethane, 2-(p,p'-dihydroxy- diphenylmethyl)benzyl alcohol, an addition product of bisphenol A and ethylene oxide, an addition product of bisphenol A and propylene oxide. It is preferred to use the polyol at 0.02 to 2 moles of the hydroxy group per mole of isocyanate group.

In forming microcapsules in this invention, a water-soluble polymer can be used and examples of water-soluble polymer used in this invention include a water-soluble anionic polymer, a water-soluble nonionic polymer and a water-soluble amphoteric polymer.

A natural anionic polymer and a synthetic anionic polymer can be used as the water-soluble anionic polymer. For example, anionic polymers having -COO- group, -S0₃- group, can be used. Specific examples of anionic natural polymers are gum arabic, alginic acid, and examples of the semisynthetic products are carboxy methyl cellulose, phthalated gelatin, sulfated starch, sulfated cellulose, ligninsulfonic acid. Also, examples of the synthetic products are maleic anhydride (including hydrolyzed derivatives) copolymers, acrylic acid (including methacrylic acid) polymers and copolymrs, vinylbenzenesulfonic acid polymers and copolymers, carboxy-denatured polyvinyl alcohol. Examples of nonionic polymers are polyvinyl alcohol, hydroxyethyl cellulose, methyl cellulose. Examples of the amphoteric anionic polymer are gelatin.

Such a water-soluble polymer is used as an aqueous solution in an amount of 0.01 to 10% by weight of the polymer. The particle size of the microcapsules is controlled to below about 20 um. If the particle size of the microcapsules is over 20 um, the quality of print images tends to be reduced. In particular, when the recording material is heated from the coated layer side by a thermal head, the particle size of the microcapsules is preferably less than 8 pm.

The microcapsules can be prepared from an emulsion containing the component or components to be encapsulated in an amount of higher than 0.2% by weight. It is also preferred for the component to permeate more smoothly through the wall of the microcapsules to encapsulate the component together with a high-boiling organic solvent as described hereinbefore.

When one or two of the diazo compound, the coupling component and the coloring activator are present in microcapsules or present in the recording layer without being encapsulated, it is preferred for the coupling component to be used in an amount of about 0.1 to about 10 parts by weight to 1 part by weight of the diazo compound and the coloring activator is used in an amount of about 0.1 to about 20 parts by weight to 1 part by weight of the diazo compound. Also, it is preferred that the diazo compound be coated in an amount of about 0.05 to about 2.0 g/m2.

When the diazo compound, the coupling component and the coloring activator used in this invention. are not encapsulated, it is preferred for each component to be in the form of a solid dispersion. In this case, each component is each dispersed in a different water-soluble polymer solution. As the water-soluble polymer used in this case, it is preferred to use the water-soluble polymer used for forming microcapsules. In this case, the concentration of the water-soluble polymer is about 2 to about 30% by weight and each of the diazo compound, the coupling component and the coloring activator is added to each solution of the water-soluble polymer at a concentration of about 5 to about 40% by weight. It is preferred that the particle size of each component thus dispersed in the solution be less than about 10 pm.

For preparing the heat sensitive recording material, a pigment such as silica, barium sulfate, titanium oxide, aluminum hydroxide, zinc oxide, calcium carbonate, and a fine powder such as styrene beads, an urea-melamine resin powder, may be used for the purposes of preventing adhesion of the recording paper to a thermal head and improving the writability. Also, for preventing adhesion. of the recording material, metal soaps, can be used. The amount of the foregoing material is about 0.2 to about 7 g/m2.

Furthermore, for preparing the heat sensitive recording material a heat melting material can be used to increase the heat recording density. The heat melting material is a material having a melting point of about 50 to about 150°C, which is in a solid state at normal temperature but is melted by heating due to the thermal heat at heat recording and thus dissolves the diazo compound, the coupling component or the coloring activator. The heat melting material is dispersed as particle of a size of about 0.1 to about 10 um and the amount used is about 0.2 to about 7 g/m² as solid. Specific examples of suitable heat melting material are fatty acid amides, N-substituted fatty acid amides, ketone compounds, N-substituted carbamate compounds, urea compounds, esters.

For making the heat sensitive recording material of this invention, the coating composition may be coated using an appropriate binder. Various emulsions of polyvinyl alcohol, methyl cellulose, carboxymethyl cellulose, hydroxypropyl cellulose, gum arabic, gelatin, polyvinylpyrrolidone, casein, styrenebutadiene latex, acrylonitrile-butadiene latex, polyvinyl acetate, polyacrylic acid ester, ethylene-vinyl acetate copolymer, can be used as the binder. The amount of the binder used is about 0.5 to 5 g/m².

The heat sensitive recording material of this invention may be further contain citric acid, tartaric acid, oxalic acid, boric acid, phosphoric acid, pyrophosphoric acid, as an acid stabilizer in addition to the foregoing compounds.

For preparing the heat sensitive recording material of this invention, a coating composition containing the diazo compound, the coupling component and the coloring activator together with, if desired, other additives as the core material of the microcapsules, a simple solid dispersion, or a solution thereof is prepared and coated on a support such as a paper, a synthetic resin film, using coating method such as a bar coating method, a blade coating method, an air knife coating method, a gravure coating method, a roll coating method, a spray coating method, a dip coating method, followed by drying to form a heat sensitive recording layer having a solid content of about 2.5 to about 15 g/m².

In other method of preparing the heat sensitive recording material of this invention, a coating composition containing the coupling component and the coloring activator as the main components together with, if desired, other components as the core Material of the microcapsules, a simple solid dispersion, or a solution thereof is prepared and coated on a support as above described followed by drying to form a pre-coated layer having a solid content of about 2 to about 10 g/m², and further a coating composition containing the diazo compound as the main component together with other additives, if any, as the main core material of the microcapsules, a simple solid dispersion, or a solution thereof is prepared and coated on the pre-coated layer followed by drying to form a diazo compound layer having a solid content of about 1 to about 10 g/m². Thus, a double layer type heat sensitive recording material is prepared. In this case, at least one of the diazo compound, the coupling component, and the color activator as the main components of the heat sensitive recording material is coated as a microencapsulated form. In a double layer type recording material, the order of the layers may be opposite to the above described embodiment. The double layers may be formed by successive coating or by simultaneous coating. The double layer type heat sensitive recording material has particularly excellent long shelf life.

In addition, in the case of using a paper as the support, it is advantageous from the standpoint of improving the shelf life of the recording material to use a neutral paper having a heat extraction pH of 6 to 9 sized with a neutral size such as an alkylketene dimer, (e.g., as decribed in JP-A-14,281/'80).

Also, for preventing the permeation of a coating liquid in a paper support and improving the contact of the heat sensitive recording layer with the thermal head, a paper having a Beck flatness of above 90 s and the following Stockigt sizing degree

as described in JP-A-116,687/'82 can be advantageously used.

Moreover, a paper having an optical surface roughness of less than 8 pm and a thickness of 40 to 75 µm described in JP-A-20,047/'82; a paper having a density of less than 0,9 g/cm³ and an optical contact ratio of higher than 15% as described in JP-A-69,0911'83; a paper capable of preventing the permeation of a coating liquid manufactured using a pulp beated above 400 ml as Canadian standard freeness (JIS P8121) as described in JP-A-69,0971'83; a paper for improving the coloring density of the resolving power using the luster surface of a base paper manufactured on a Yankee paper machine as a coating surface as described in JP-A-65,6951'83; a paper having improved coatability by appiyng a corona discharging treatment to a base paper as described in JP-A-145,8721'82, can be used in this invention with good results. Thus, these supports used in general in the field of ordinary heat sensitive recording papers can be used as support in this invention.

The heat sensitive recording material prepared according to this invention can be used as printer papers for facsimile and computers requiring high-speed rcording and can be fixed by exposing the recording material to light, after heat printing, to decompose the unreacted diazo compound. Furthermore, the heat sensitive recording material can be used as a heat developable copying paper.

The invention is explained below in greater detail by reference to the following examples but the invention is not to be construed limited to these examples. In addition, the "part" for the addition amount is "by part by weight".

### Examples 1 to 5 and Comparison Examples 6 to 8

Using following Diazo Compounds (1) to (3) each of the diazo compound in an amount shown in Table 1 below and 10 parts of the addition product of xylylene diisocyanate and trimethylolpropane (3:1 by weight) were dissolved in a mixture of 20 parts of dibutyl phthalate and 5 parts of ethyl acetate. The solution of the diazo compound was mixed with an aqueous solution of 3.5 parts of polyvinyl alcohol, 1.7 parts of gelatin, and 3.6 parts of 1,5-dihydroxypentane dissolved in 58 parts of water and the mixture was an emulsion dispersion at 20°C to provide an emulsion having a mean particle size of 3 um. To the emulsion was added 100 parts of water and the mixture was heated to 40 to 70°C with stirring. Thus, after 2 hours, three kinds of capsule-containing solutions containing the diazo compound as the core material of the microcapsules were obtained.

### Diazo Compound (1)

Diazo Compound (2) Diazo Compound (3)

Each of the dispersions of coupling components (1) to (3) shown below having a mean particle size of about 3 pm was obtained by dispersing 20 parts of each coupling component and 5 parts of polyvinyl alcohol in 100 parts of water for about 24 hours using a sand mill.

### Coupling Component (1):

2-hydroxy-3-naphthoeic acid morpholinopropylamide

### Coupling Component (2):

2-hydroxynaphthoeic acid anilide

### Coupling Component (3):

2-Hydroxy-3-naphthoeic acid-2'-methylanilide

Then, 20 parts of triphenyl guanidine and 5 parts of polyvinyl alcohol were dispersed in 100 parts of water for about 24 hours using a sand mill to provide a dispersion of triphenyl guanidine having a mean particle size of about 3 pm.

Then, 50 parts of the liquid of the capsules of the diazo compound thus obtained, 15 parts of the dispersion of the coupling component, and 15 parts of the dispersion of triphenyl guanidine were added to 20 parts of an aqueous solution of 5% zinc stearate to provide a coating liquid. Each of the coating liquids was coated on a smooth wood free paper (50 g/m²) at a dry coverage of 14 g/m² using coating rod and dried for 30 minutes at 45°C to provide Heat Sensitive Recording Materials (1) to (5). The kind and addition amount of the diazo compound used and the kind of the coupling component are shown in Table 1 below.

On the other hand, for the sake of comparison, Heat Sensitive Recording Materials (6) to (8) were prepared as comparison samples. That is; a dispersion of a diazo compound having a mean particle size of 3 um was prepared by adding an appropriate amount of the diazo compound and 5.2 parts of polyvinyl alcohol to 93.8 parts of water and dispersing the diazo compound for about 24 hours using a sand mill. Then, 25 parts of the dispersion of the diazo compound thus prepared, 15 parts of the dispersion of a coupling component prepared in the same manner as above described, and 15 parts of the dispersion of triphenyl guanidine prepared in the same manner as above described were added to 20 parts of a solution of 5% zinc stearate to provide a coating liquid. Each of the coating liquids thus prepared was coated on a smooth wood free paper as above described to provide comparison Heat Sensitive Recording Materials (6) to (8).

Furthermore, for comparison, Heat Sensitive Recording Materials (9) to (11) were prepared as comparison samples by following the same procedure as described above for preparing Heat Sensitive Recording Materials (1) to (5) except that each diazo compound was microencapsulated by the method shown in Example 1 of JP―A―192,944/'82.

The kinds and the amounts of the diazo compounds and the coupling components used in the above comparison examples are shown in Table 1 below.

Heat Sensitive Recording Materials (1) to (11) thus prepared were employed in heat recording using a recording machine, G II Mode (Panfax 7200)^{@} made by Matsushita Denso K.K. and then each sample was fixed by an overall light exposure to the sample using a copying machine, Ricopy High Start Type 4^{@}, made by Ricoh Company, Ltd. The blue density of the recorded images thus obtained was measured using a Macbeth reflection densitometer. The results obtained are shown in Table 1 below.

On the other hand, when heat recording was employed again in the fixed area of each sample, no image was recorded and hence it was confirmed that each sample was completely fixed.

Then, to determine the shelf life of each sample, the background density (fog) of each of Heat Sensitive Recording Materials (1) to (11) and the fog of each sample after storing each sample in the dark under the conditions of 50°C and 90% relative humidity for forced deterioration testing were measured to evaluate change of fog. The results obtained are also shown in Table 1 below.

As is clear from the results shown in Table 1 above, it can be seen that the image density of the samples of this invention is high as that of the comparison samples in which the diazo compound was not encapsulated and is higher than that of the comparison samples in which the diazo compound encapsulated according to the method of JP-A-192,944/'82. Also the increase of fog after the forced deterioration test is less in the samples of this invention, which shows the samples of this invention have a very excellent shelf life as compared with the comparison examples.

### Examples (12) to (16) and Comparison Examples (17) to (19)

By following the same procedures described previously for Heat Sensitive Recording Materials (1) to (5), a capsule liquid of a coupling component was prepared by adding 5 parts of the coupling component in place of adding the diazo compound and also a dispersion of a diazo compound was prepared by adding an appropriate amount of a diazo compound in place of adding 20 parts of the coupling component.

Then, a coating liquid composed of 50 parts of the capsule liquid of the coupling component, 15 parts of the dispersion of the diazo compound, 15 parts of a dispersion of triphenyl guanidine prepared in the same manner as in the foregoing examples, and 20 parts of a 5% zinc stearate aqueous solution was coated as in Examples (1) to (5) to provide Heat Sensitive Recording Materials (12) to (16) as samples of this invention. The kind and addition amount of the diazo compound and the kind of the coupling component used in each example are shown in Table 2 below.

On the other hand, for comparison, Heat Sensitive Recording Materials (17) to (19) were prepared as comparison samples by employing the capsule wall-forming method described in Example 1 of JP-A-192,244/'82, i.e. a method using a polymer for forming capsule walls in place of forming the wall by the polymerization of reactants as in this invention. That is, in 50 parts of cyclohexane were dissolved 10 parts of a copolymer of vinyl acetate, butyl methacrylate, and styrene and then 5 parts of a coupling component, and a solution composed of 5.2 parts of polyvinyl alcohol and 8.4 parts of water was added to the solution. The mixture was stirred at high speed and at room temperature (about 20 to 30°C) to form an emulsified dispersion and then cyclohexane was distilled off from the dispersion at reduced pressure with stirring to provide a capsule liquid of the coupling component. Then, the capsule liquid was filtered, washed with water, and dried in vacuum to provide a capsule powder. A coating liquid was prepared by adding 5 parts of the capsule powder thus obtained in place 50 parts of the capsule liquid of the coupling component for the coating liquid used in the case of preparing Heat Sensitive Recording Materials (12) to (16) and the coating liquid was coated as in the case of Examples (1) to (5). Thus, comparison Heat Sensitive Recording Materials (17) to (19) were prepared. The kind and amounts of the diazo compound and the kind of the coupling component used in the above comparison examples are shown in Table 2 below.

About the Heat Sensitive Recording Materials (12) to (19) thus prepared, the measurement of the recorded image density and the measurement of fog before the forced deterioration test and fog after the forced deterioration test were performed as in Examples (1) to (5) and Comparison Examples (6) to (11). The results thus obtained are shown in Table 2 below.

Also, when heat recording was applied again to the fixed area of each of Heat Sensitive Recording Materials (12) to (19), no image was recorded, which showed the samples were completely fixed.

As is clear from the results shown in Table 2 above, the samples of this invention wherein the coupling component was emulsified as the core material and then the capsule wall composed of a polymer was formed by polymerizing the reactants around the core material gave high image density as compared to the comparison samples wherein the microcapsules were prepared by dissolving a previously polymerized polymer and the increase of fog after the forced deterioration testing is less in the samples of this invention as compared to the comparison samples, which shows the excellent shelf life of the samples of this invention.

### Example 20

By following the same procedure of preparing the capsule liquid in Examples (1) to (5) except that 5 parts of 2-phenyl-4-methylimidazole was added in place of the diazo compound used in these examples, a capsule liquid was prepared. Then, a coating liquid was prepared by adding 50 parts of the capsule liquid thus obtained, 15 parts of the dispersion of coupling component (1) prepared in the same manner as in Examples (1) to (5), and 15 parts of the dispersion of diazo compound (1) prepared in the same manner as in Examples (1) to (5) to 20 parts of a 5% zinc stearate aqueous solution. By coating the coating solution as in Examples (1) to (5), Heat Sensitive Recording Material (20) was prepared and tested as in the foregoing examples. The results obtained are shown in Table 3 below.

### Example 21

By following the method of preparing the capsule liquid as in Examples (1) to (5) except that 1 part of diazo compound (1) and 1 part of coupling component (2) were added in place of the diazo compound used in the foregoing examples, a capsule liquid was prepared. A coating liquid was prepared by adding 65 parts of the capsule liquid thus obtained and 20 parts of the dispersion of triphenyl guanidine prepared by the same manner as in Examples (1) to (5) to 15 parts of a 5% zinc stearate aqueous solution and coated as in the foregoing examples to provide Heat Sensitive Recording Material (21). The sample was also tested as in the foregoing examples. The results obtained are shown in Table 3 below.

As is clear from the results shown in Table 3 above, Heat Sensitive Recording Materials (20) and (21) of this invention each containing a part of the main components in the microcapsules show high image density and less increase of fog after the forced deterioration testing, which shows the excellent shelf life of the samples.

### Example 22

By following the same method of preparing the capsuleliquid of the diazo compound as in Examples (1) to (5) except that 5 parts of the addition product of xylylene diisocyanate and trimethylol propane (3:1 by weight) and 5 parts of an addition product of tolylene diisocyanate and trimethylolpropane (3:1 by weight) were used in place of 10 parts of the addition product of xylylene diisocyanate and trimethylolpropane, a capsule liquid of diazo compound (1) as the core material was prepared. Then, a coating liquid was prepared by adding 50 parts of the capsule liquid thus prepared, 15 parts of the dispersion of coupling component (1) prepared in the same manner as in Examples (1) to (5), and 15 parts of the dispersion of triphenyl guanidine prepared in the foregoing examples to 20 parts of a 5% zinc stearate aqueous solution and coated as in the foregoing examples to provide Heat Sensitive Recording Material (22). When the sample was tested as in Examples (1) to (5), the image density was 1.3 and the fog before and after the forced deterioration testing was 0.08 and 0.13, respectively. That is, the sample showed a high image density and excellent shelf life.

### Example 23

The same method as used in preparing the capsule liquid in Examples 1 to 5was followed except that a solution of 5.2 parts of polyvinyl alcohol and 2.5 parts of hexamethylenediamine dissolved in 58 parts of water was used in place of the aqueous polyvinyl alcohol solution for emulsifying the solution of the diazo compound. A coating liquid was prepared by adding 50 parts of the capsule liquid of diazo compound (1) thus prepared, 15 parts of the dispersion of coupling component (1), and 15 parts of the dispersion of triphenyl guanidine to 20 parts of a 5% zinc stearate aqueous solution and coated as in Examples 1 to 5 to provide Heat Sensitive Recording Material (22). When the sample was tested as in the foregoing examples, the image density was 1.1 and the fog before and after the forced deterioration testing was 0.08 and 0.13, respectively. Thus, the sample showed a high image density and excellent shelf life.

### Example 24

By following the same procedure as in Example 23 except that 0.2 part of terephthalic acid chloride was further added to the solution containing the diazo compound as the core material in the method of preparing the capsule liquid in Example 23, Heat Sensitive Rcording Material (24) was prepared. The capsule wall in this case was composed of polyurea and polyamide. When the sample was tested as in Examples 1 to 5, the image density was 1.1 and the fog before and after the forced deterioration testing was 0.08 to 0.1, respectively, which showed the excellent shelf life of the sample.

## Claims

1. A process for preparing a heat sensitive recording material comprising a support having thereon a recording layer containing (a) a diazo compound, (b) a coupling component and (c) a coloring activator, wherein at least one of said diazo compound (a), said coupling component (b) and said coloring activator (c) is present in microcapsules as the core material with the proviso that all three components (a) to (c) are not present in the same microcapsules, and the wall of said microcapsules is formed of a polymer, characterized in that the core material is dispersed in one or more reactants and the obtained dispersion is then subjected to a polymerisation reaction whereby the wall of said microcapsules is formed around the core material.

2. The process according to claim 1, characterized in that as material of the wall of the microcapsules a polyurethane, polyurea, polyamide or polyester is used.

3. The process according to claim 1 or 2, characterized in that one of the three components (a) to (c) is included in microcapsules and the component included in the microcapsules is the diazo compound (a) and the wall of the microcapsules is composed of a polymer formed around the material encapsulated by polymerization of at least one polyhydric isocyanate as a first wall-forming material and at least one polyol as a second wall-forming material capable of forming a polymer by reaction with the polyhydric isocyanate.

4. The process according to any of claims 1 to 3, characterized in that two of the three components (a) to (c) are included in microcapsules.

5. The process according to claim 4, characterized in that said two components are included in the same microcapsules.

6. The process according to claim 5, characterized in that said two components are included in different microcapsules.

7. The process according to any of claims 1 to 6, characterized in that each of said three components (a) to (c) is included in different microcapsules.

8. The process according to any of claims 1 to 7, characterized in that said three components (a) to (c) are included in microcapsules, two components being included in the same microcapsules and the other component being included in other microcapsules.

9. The process according to any of claims 1 to 8, characterized in that the material encapsulated is included in microcapsules together with an organic solvent.

10. The process according to claim 9, charcterized in that said organic solvent is a water-insoluble high-boiling solvent having a boiling point higher than 180°C.

11. The process according to claim 10, characterized in that said organic solvent is a phosphoric acid ester, a phthalic acid ester, a carboxylic acid ester, a fatty acid amide, an alkylated biphenyl, an alkylated terphenyl, a chlorinated paraffin, or a diarylethane.

12. The process according to any of claims 1 to 11, characterized in that the diazo compound is represented by the general formula wherein Ar represents a substituted aromatic moiety and X- represents an acid anion containing a perfluoroalkyl group or an acid anion containing a perfluoroalkenyl group.

13. The process according to any of claims 3 to 12, characterized in that the polyol is selected from the polyols having the following groups (I), (II), (III) or (IV) between the two hydroxy groups in the molecular structure:
(I) aliphatic hydrocarbon group having 2 to 8 carbon atoms wherein Ar' in groups (II), (III) and (IV) represents an unsubstituted or substituted aromatic moiety and the aliphatic hydrocarbon group of (I) has the moiety -CₙH₂ₙ₋ (wherein n is 2 to 8) as the fundamental skeleton and the hydrogen atom may be replaced by another element.

## Patentansprüche

1. Verfahren zur Herstellung eines wärmeempfindlichen Aufzeichnungsmaterials mit einem Träger und einer darauf aufgebrachten Aufzeichnungsschicht, die enthält (a) eine Diazoverbindung, (b) eine kuppelnde Komponente und (c) einen färbenden Aktivator, wobei. mindesten ein Vertreter aus der Gruppe der Diazoverbindung (a), der kuppelnden Komponente (b) und des färbenden Aktivators (c) in Mikrokapseln als Kernmaterial vorliegt mit der Maßgabe, daß nicht alle 3 Komponenten (a) bis (c) in den gleichen Mikrokapseln vorliegen und die Wand der Mikrokapseln aus einem Polymeren besteht, dadurch gekennzeichnet, daß das Kernmaterial in einem oder mehr Reaktanten dispergiert wird und die erhaltene Dispersion dann einer Polymerisationsreaktion unterworfen wird, wodurch die Wand der Mikrokapseln um das Kernmaterial herum gebildet wird.

2. Verfahren nach Anspruch 1, dadurch gekennzeichnet, daß als Material für die Wand der Mikrokapseln ein Polyurethan, ein Polyharnstoff, ein Polyamid oder ein Polyester verwendet wird.

3. Verfahren nach Anspruch 1 oder 2, dadurch gekennzeichnet, daß eine der 3 Komponenten (a) bis (c) in Mikrokapseln eingeschlossen ist und die in den Mikrokapseln eingeschlossene Komponente die Diazoverbindung (a) ist, und daß die Wand der Mikrokapseln besteht aus einem Polymeren, das gebildet worden ist durch Polymerisation mindestens eines Polyhydroxyisocyanats als einem ersten wandbildenden Material und mindestens eines Polyols als einem zweiten wandbildenden Material, das durch Umsetzung mit dem Polyhydroxyisocyanat ein Polymeres bilden kann, um das eingekapselte Material herum.

4. Verfahren nach einem der Ansprüche 1 bis 3, dadurch gekennzeichnet, daß zwei der drei Komponenten (a) bis (c) in Mikrokapseln eingeschlossen sind.

5. Verfahren nach Anspruch 4, dadurch gekennzeichnet, daß diese beiden Komponenten in den gleichen Mikrokapseln eingeschlossen sind.

6. Verfahren nach Anspruch 5, dadurch gekennzeichnet, daß diese beiden Komponenten in verschiedenen Mikrokapseln eingeschlossen sind.

7. Verfahren nach einem der Ansprüche 1 bis 6, dadurch gekennzeichnet, daß jde der drei Komponenten (a) bis (c) in verschiendenen Mikrokapseln eingeschlossen ist.

8. Verfahren nach einem der Ansprüche 1 bis 7, dadurch gekennzeichnet, daß die dri Komponenten (a) bis (c) in Mikrokapseln eingeschlossen sind, wobei zwei Komponenten in den gleichen Mikrokapseln eingeschlossen sind und die andere Komponente in anderen Mikrokapseln eingeschlossen ist.

9. Verfahren nach einem der Ansprüche 1 bis 8, dadurch gekennzeichnet, daß das eingekapselte Material zusammen mit einem organischen Lösungsmittel in Mikrokapseln eingeschlossen ist.

10. Verfahren nach Anspruch 9, dadurch gekennzeichnet, daß es sich bei dem organischen Lösungsmittel um ein in Wasser unlösliches hochsiedendes Lösungsmittel mit einem Siedepunkt von mehr als 180°C handelt.

11. Verfahren nach Anspruch 10, dadurch gekennzeichnet, daß es sich bei dem organischen Lösungsmittel um einen Phosphorsäureester, einen Phthalsäureester, einen Carbonsäureester, ein Fettsäureamid, ein alkyliertes Biphenyl, ein alkyliertes Terphenyl, ein chloriertes Paraffin oder ein ^{p}iarylethan handelt.

12. Verfahren nach einem der Ansprüche 1 bis 11, dadurch gekennzeichnet, daß die Diazoverbindung dargestellt wird durch die allgemeine Formel worin Ar einen substituierten aromatischen Rest darstellt und X- ein eine Perfluoroalkylgruppe enthaltendes Säureanion oder ein eine Perfluoroalkenylgruppe enthaltendes Säureanion darstellt.

13. Verfahren nach einem der Ansprüche 3 bis 12, dadurch gekennzeichnet, daß das Polyol ausgewählt wird aus den Polyolen, die zwischen den beiden Hydroxygruppen in der Molekülstruktur die folgenden Gruppen (1), (11), (111) oder (IV) aufweisen:
(I) aliphatische Kohlenwasserstoffgruppe mit 2 bis 8 Kohlenstoffatomen worin Ar' in den Gruppen (11), (111) und (IV) einen unsubstituierten oder substituierten aromatischen Rest darstellt und die aliphatische Kohlenwasserstoffgruppe von (I) den Rest -CₙH₂ₙ- (worin n = 2 bis 8) als Grundgerüst aufweist und das Wasserstoffatom durch ein anderes Element ersetzt sein kann.

## Revendications

1. Procédé pour préparer un matériau d'enregistrement sensible à la chaleur comprenant un support portant une couche d'enregistrement contenant (a) un composé diazo, (b) un composant de couplage et (c) un activateur de coloration, dans lequel l'un au moins dudit composé diazo (a), dudit composant de couplage (b) et dudit activateur de coloration (c) est présent en microcapsules comme matériau constituant le noyau, avec la réserve que les trois composants (a) à (c) ne sont pas présents dans les mêmes microcapsules, et la paroi desdites microcapsules est formée d'un polymère, caractérisé en ce que le matériau constituant le noyau est dispersé dans on ou plusieurs réactifs et la dispersion obtenue est ensuite soumise à une réaction de polymérisation par laquelle la paroi desdites microcapsules est formée autour du matériau constituant le noyau.

2. Le procédé selon la revendication 1, caractérisé en ce qu'on utilise un polyuréthanne, une polyurée, un polyamide ou un polyester comme matériau de la paroi des microcapsules.

3. Le procédé selon la revendication 1 ou 2, caractérisé en ce que l'un des trois composants (a) à (c) est inclus dans des microcapsules et le composant inclus dans les microcapsules est le composé diazo (a) et la paroi des microcapsules est composée d'un polymère formé autour du matériau encapsulé par polymérisation d'au moins un isocyanate polyhydrique comme premier matériau formateur de paroi et d'au moins un polyol comme second matériau formateur de paroi capable de former un polymère par réaction avec l'isocyanate poIyhydrique.

4. Le procédé selon l'une quelconque des revendications 1 à 3, caractérisé en ce que deux des trois composants (a) à (c) sont inclus dans des microcapsules.

5. Le procédé selon la revendication 4, caractérisé en ce que lesdits deux composants sont inclus dans les mêmes microcapsules.

6. Le procédé selon la revendication 4, caractérisé en ce que lesdits deux composants sont inclus dans des microcapsules différentes.

7. Le procédé selon l'une quelconque des revendications 1 à 6, caractérisé en ce que chacun desdits trois composants (a) à (c) est inclus dans des microcapsules différentes.

8. Le procédé selon l'une quelconque des revendications 1 à 7, caractérisé en ce que lesdits trois composants (a) à (c) sont inclus dans des microcapsules, deux composants étant inclus dans les mêmes microcapsules et l'autre composant étant inclus dans d'autres microcapsules.

9. Le procédé selon l'une quelconque des revendications 1 à 8, caractérisé en ce que le matériau encapsulé est inclus dan des microcapsules avec un solvant organique.

10. Le procédé selon la revendication 9, caractérisé en ce que ledit solvant organique est un solvant à haut point d'ébullition insoluble dans l'eau ayant un point d'ébullition supérieur à 180°C.

11. Le procédé selon la revendication 10, caractérisé en ce que ledit solvant organique et un ester d'acide phosphorique, un ester d'acide phtalique, un ester d'acide carboxylique, un amide d'acide gras, un biphényle alkylé, un terphényle alkylé, une paraffine chlorée, ou un diaryléthane.

12. Le procédé selon l'une quelconque des revendications 1 à 11, caractérisé en ce que ledit composé diazo est représenté par la formule générale dans laquelle Ar représente un reste aromatique substitué et X- représente un anion acide contenant un groupe perfluoroalkyle ou un anion acide contenant un groupe perfluoroalcényle.

13. Le procédé selon l'une quelconques des revendications 3 à 12, caractérisé en ce que le polyol est choisi parmi les polyols ayant les groupes (I), (II), (III) ou (IV) suivants entre les deux groupes hydroxy dans la structure moléculaire:
(I) groupe aliphatique hydrocarboné ayant 2 à 18 atomes de carbone dans lesquelles Ar' dans les groupes (II), (III) et (IV) représente un reste aromatique substitué ou insubstitué et le groupe hydrocarboné aliphatique de (I) possède le reste―CₙH₂ₙ― (où n est 2 à 8) comme squelette de base et l'atome d'hydrogène peut être remplacé par un autre élément.
